

Patented Aug. 17, 1943

2,326,837

## UNITED STATES PATENT OFFICE

2,326,837

CLEANING COMPOSITION AND METHOD  
FOR ITS USETimothy J. Coleman, Buffalo, N. Y., assignor to  
National Carbon Company, Inc., a corporation  
of New YorkNo Drawing. Application January 13, 1940,  
Serial No. 313,727

10 Claims. (Cl. 252—142)

This invention relates to the cleaning of metal surfaces; and to a composition and method for its use that is particularly adapted for removing scale, rust, and other oxide formations, and deposits or films of grease and oil, from the surfaces of heat-exchange equipment, such as the cooling systems of internal combustion engines.

The composition of the invention has especial utility for the removal of scale, rust, oil and grease deposits, etc. from the heat-exchange surfaces of present-day internal combustion engines, portions of which surfaces are formed of aluminum, brass, copper, tin, solder, and other non-ferrous metals subject to ready attack by acidic reagents in aqueous solution.

It is well known that considerable corrosion normally occurs in the cooling systems of internal combustion engines even when water alone is used as the cooling agent. This corrosion is often intensified when certain types of antifreeze compounds are used in such systems; so that the radiator tubes become more or less clogged with scale and rust. Grease and oil which may enter the cooling fluid at the circulation pump deposit on the radiator tubes and other parts and help to bond these solids thereto.

Many preparations for periodically removing these undesirable deposits from cooling systems have been tried. Many of them are alkaline, and usually contain caustic alkalies, sodium carbonate, tri-sodium phosphate, or sodium silicate.

The advent of aluminum cylinder heads has rendered such alkaline cleaning compounds objectionable because of the rapid attack of aluminum by alkaline solutions. Furthermore, where organic antifreeze compounds are used, the presence of even small amounts of alkaline silicates causes the formation of an insoluble gel which increases the radiator clogging effect. Such cleaners have no action upon rust coatings or upon rust itself; nor have they powers of loosening iron oxide scale from the metal.

Acid cleaning compositions are extremely effective for removing oxide scale. However, the common acids readily attack aluminum as well as iron, brass, copper, and various other metals used in heat-exchange apparatus. Moreover, the usual acid compositions are not capable of removing grease and oil present upon the metal surfaces.

The present invention is based in important part upon the discovery that by the employment of certain mixtures of solid compounds, herein-after more fully described, stable acidic cleaning

composition may be produced which, in solution in water or other solvent, is highly effective for removing from a heat-exchange system rust, scale, and other solid impurities, together with grease and oil, while preventing or inhibiting undesirable attack by the acidic components upon parts of the system made of such non-ferrous metals as aluminum, brass, copper, tin and lead.

Among the more important objects of the invention are: To provide a novel composition and method adapted to remove scale, rust, grease, oils and the like from metal surfaces of heat-exchange systems made of iron, steel, aluminum, brass, copper, lead, tin, or alloys containing one or more of these or similar metals, and which will leave the metal surfaces clean and corrosion-resistant; to provide a novel acidic cleaning composition in dry or solid state, which is stable in storage and is readily soluble in water and aqueous solutions; to provide a novel acidic composition for cleaning metal surfaces, and which is emulsifiable with oil and grease in an acid state, and which inhibits or retards the corrosion by the acidic component of aluminum, copper, and alloys containing copper and/or tin and/or zinc.

In its broadest scope the invention involves the preparation and use of a novel cleaning composition which preferably is preparable in the state of a dry or solid mixture, and which comprises (1) an acidic agent capable of dissolving rust and of loosening and removing scale and metallic oxide coatings from metal surfaces; (2) an organic compound of the type hereinafter described, capable of functioning as an emulsifying agent for oils and greases in an acid, a neutral, or an alkaline medium; and (3) an agent which effectively inhibits or retards the attack by the said acidic agent upon those portions of a heat-exchange system made of aluminum, brass, copper, tin, lead, and alloys thereof.

Although any solid water-soluble acid, or a water-soluble compound capable upon hydrolysis of yielding an acid, or mixtures of such substances, may be used as the active cleaning agent, it is preferred to use a compound which is stable in the dry state and is readily miscible with the other solid ingredients in finely-divided form. One example of such agent is sodium bisulfate. However, many other water-soluble solid acidic compounds may be used advantageously, among which are other acid salts, such as mono-sodium acid phosphate; and oxalic and citric acids.

As the water-soluble emulsifying agent, there may be used a wide variety of organic compounds,

including the sulfonates and sulfate esters produced by the sulfonation or sulfation of various saturated and unsaturated organic compounds having six or more carbon atoms in their molecules, such as aliphatic and aromatic monohydric and polyhydric alcohols, fatty acids, amines, naphthenic acids, hydroxy fatty acids and esters derived therefrom; and salts derived from these sulfonates and sulfate esters by treatment with a base.

Among emulsifying agents suitable for use may be mentioned fatty acid esters of polyhydroxy aliphatic compounds and derivatives thereof such as diglycol oleate, diglycol stearate, and condensation products of fatty acids with glycerine or with derivatives of these hydroxy compounds, such as ethylene glycol monoalkyl ethers; hydroxy alkyl amines and derivatives thereof, such as the ethanolamine soaps, and sulfonates thereof, and the condensation products of such amines with alkylene oxides, halohydrins and sulfonates; alkyl amine halides such as cetylamine hydrochloride, cetyltriethylamine hydrochloride, and cetyltriethyl ammonium iodide; sulfonated substituted amides of carboxylic acids, such as the sodium salt of the amino-derivative of oleic acid and amino-ethane-sulfonic acid; amides of aliphatic acid sulfates and sulfonates; benzene sulfonic acid salts and esters, amides, and alkylated derivatives thereof; naphthalene sulfonic acid salts and esters, amides, and alkylated derivatives thereof; phenol sulfonic acid salts and esters, amides, and alkylated derivatives thereof; naphthol sulfonic acid salts and esters, amides, and alkylated derivatives thereof; and cresol sulfonic acid salts, and esters, amides, and alkylated derivatives thereof.

The products derived by the sulfonation or sulfation of saturated branched-chain secondary alcohols having eight to seventeen or more carbon atoms in the molecular structure, and salts and esters derived therefrom are highly efficacious emulsifying agents when present in the composition in small amounts. These alcohols may be produced by the hydrogenation of unsaturated ketones which, in turn, are derived from the products of the condensation of aliphatic ketones such as acetone with aliphatic aldehydes such as ethylhexaldehyde, by removal of the elements of water. Examples of such agents are the sodium and the mono- and triethanolamine derivatives of the sulfate esters of 7-ethyl-2-methylundecanol-4; of 3-ethylundecanol-6; of 5-ethylnonanol-2; and of 3,9-diethyltridecanol-6.

Especially effective as emulsifying agents in the cleaning composition are the water-soluble salts of sulfonated derivatives of alkylated phenols and benzines of the respective types designated by the formulae



and



wherein A designates either hydrogen or the methyl group; R designates an alkyl group containing at least nine carbon atoms, and prefer-

ably containing between nine and sixteen carbon atoms; and M designates either hydrogen, an alkali metal, an alkaline earth metal, an ammonium or an organic amino group. Examples of such emulsifying agents are the mixtures of the sodium derivatives of alkylated phenol—or mixtures of the corresponding derivatives of alkylated benzene—the components of the respective mixtures having a composition corresponding to the respective formulae



and



wherein R designates an alkyl group having between nine and sixteen carbon atoms. The alkyl groups in the mixtures of these alkylated compounds preferably average around fourteen carbon atoms.

Such products may be made, for example, by chlorinating under pressure the kerosene fraction of a paraffin base mineral oil, condensing the resultant mixture of alkyl chlorides with phenol in the presence of zinc chloride as a condensing agent or catalyst, sulfonating the resultant alkylated phenol in well-known manner with a sulfonating agent such as fuming sulfuric acid or chlorsulfonic acid, and neutralizing with a water-soluble base such as sodium hydroxide or carbonate, the sulfonated product thus obtained. The original kerosene fraction has a specific gravity between 0.78 and 0.80; whereas the chlorinated kerosene may have a specific gravity between 0.91 and 0.925.

If desired, the kerosene fraction may be fractionated to separate it into selected fractions; the selected fraction halogenated in the manner indicated; and the halogenated product further treated to produce the salt of the sulfonated derivative thereof.

The above-mentioned sodium sulfonates of alkylated phenol—or mixtures of said sulfonates—which, for convenience, will be designated hereinafter as the sodium sulfonate of tetradecyl phenol—are solids, soluble in water, and contain around equal parts of the said sulfonate and of sodium sulfate. In an acid solution it also gives some corrosion resistance to non-ferrous metals of the type mentioned above. This protection, when afforded in connection with the use of acid solutions also containing phosphates, as herein-after described, is greatest when the ratio of the sodium sulfonate of tetradecyl phenol to the phosphate group is around two or three to one. Some production is afforded even outside these limits. By maintaining the ratio of said sulfonate to the phosphate group within the limits indicated, substantially no electrolytic corrosion of brass surfaces exposed to the liquid occurs.

One procedure for producing a water-soluble sulfonate of an alkylated benzene is as follows: A commercial kerosene fraction of a paraffin base mineral oil is refractionated; and the fraction containing the hydrocarbons within the range from octane to hexadecane is chlorinated. The mixtures of alkyl chlorides thus formed are condensed with benzene in the presence of zinc chloride or aluminum as a catalyst, and

the resultant mixtures of alkylated benzenes are sulfonated in the usual manner with concentrated sulfuric acid or chlorosulfonic acid. The sulfonation product is then neutralized by means of a water-soluble base, such as sodium hydroxide or carbonate, ammonia or an amine. A procedure of this type is disclosed in United States Patent 2,161,174 of L. P. Kyrides.

It is well known that any acidic reagent capable of readily removing scale, rust and other oxides from ferrous and non-ferrous metal surfaces must attack such surfaces. Indeed, inhibitors effective for protecting ferrous metal from undue corrosion frequently do not inhibit the attack of cooling system parts made of aluminum and other non-ferrous metals.

It now has been discovered that the presence in the composition of a small amount of a water-soluble phosphate such as the ammonium and alkali metal phosphates, in conjunction with the said emulsifying agent, which also possesses some corrosion-inhibiting action, affords splendid protection for non-ferrous metal surfaces. A basic phosphate, such as secondary ammonium phosphate, has been found especially effective for inhibiting the action of the acidic component upon aluminum, aluminum alloys, and copper and copper alloys. A portion of the phosphate, if desired, may be replaced with other substances having a somewhat similar action, such as a water-soluble cyanate; or "Phosphine G. N.", the latter of which is a yellow-brown dye readily available on the market under this trade name.

When using an acidic salt containing substantial amounts of chlorides or nitrates, it is desirable to increase somewhat the amount of inhibitor used, since the efficiency of the latter may be somewhat reduced in the presence of these salts.

The components of the cleaning composition preferably are mixed in the dry state. Alternatively, the composition can be prepared in the form of a solution thereof in water or a water-soluble solvent, followed by evaporation of the liquid. The dry mixtures are readily prepared, are stable in storage, and are readily and safely transported.

A mixture containing 84.5% by weight of finely-divided sodium bisulfate, about 6% of the aforesaid finely-divided sodium sulfonate derivative of tetradecyl phenol, about 5% of sodium sulfate, and 4.2% of dibasic ammonium phosphate provides these solid ingredients in proportions such that, when the mixture is dissolved in water to yield dilute solutions containing the acidic ingredient within the range of concentrations hereinafter specified, the other ingredients will be present in amounts sufficient to insure their functioning in the manner described.

In utilizing the invention, preferably sufficient of the composition is mixed with water, or its equivalent, to provide a liquid having an effective free acid concentration of from 0.1% to 10%. A concentration of from .01% to 1% of the water-soluble emulsifying agent ordinarily is required, depending largely upon the amount and nature of the oil and/or grease that must be emulsified.

The amount of the phosphate or other inhibitor depends upon the presence or absence of non-ferrous metals readily attackable by the acid solutions. Generally around .15% of the inhibitor in the said liquid is sufficient, though more or less than this amount can be employed. The phosphate ion, in concentrations of from .05% to 0.5% or more of the solution, effectively inhibits the corrosion of the non-ferrous metals hereinbefore named.

In use, a solution of the cleaning composition in water, alcohol, or other suitable vehicle, is contacted with the metal surfaces to be cleaned, preferably in the heated state. Thus, in cleaning the cooling system of an internal combustion engine, an aqueous solution of the said composition is circulated through the cooling system while running the engine, thus heating the solution to around 175° F. After such operation, which may last for from fifteen minutes to several hours or more, the cleaning solution is withdrawn, and the system is flushed and refilled with clean hot water once or twice.

Preferably the water used for the first flushing contains a neutralizing agent such as sodium carbonate in amount sufficient to neutralize all traces of residual acidic substance. This treatment with neutralizing agent particularly is desirable when the cooling system subsequently is to be filled with an antifreeze compound or other liquid containing an alkaline component.

The following examples serve to illustrate the invention:

**Example 1**

An aqueous solution containing 3% sodium bisulfate, 0.4% of the aforesaid sodium sulfonate derivative of tetradecyl phenol (containing approximately 44% of the said sulfonate, 55.5% of sodium sulfate, and 0.5% of zinc sulfate), and 0.15% of dibasic ammonium phosphate, was circulated at a temperature of around 175° F. through the cooling system of an internal combustion engine for about one hour. The solution then was withdrawn, and the system was flushed with a dilute aqueous solution of sodium carbonate slightly in excess of that required to neutralize the residual acid present. This solution then was withdrawn and the system was flushed with clean water. This assisted in removing loose rust particles and in rinsing out dissolved iron oxide that had been reprecipitated by the carbonate. The metal parts of the system were effectively cleaned of scale, rust, and oily materials by the treatment.

**Example 2**

An aqueous solution containing 3% of sodium bisulfate; 0.25% of the sodium salt of the sulfate ester of tetradecanol-4, (produced in the manner described in United States Patent 2,088,014 of J. N. Wickert and B. T. Freure); and about 0.15% of secondary ammonium phosphate; was prepared by dissolving in water a mixture of 480 parts of sodium bisulfate, 64 parts of the said sodium salt, and 24 parts of secondary ammonium phosphate—all parts by weight. This solution was circulated at a temperature around 175° F. through a radiator, in the general manner described in Example 1, and was then withdrawn and the radiator flushed in the manner described in that example. The metal parts were effectively cleaned of rust, scale, and oily materials.

Similar solutions wherein the said emulsifying agent was replaced with an equal quantity of sodium octyl sulfate were somewhat less effective for removing grease from the radiator, and for assisting the inhibitor to protect non-ferrous surfaces from corrosion.

**Example 3**

There was prepared an aqueous solution similar to that described in Example 1, with the ex-

ception that 0.4% of the sodium salt of monosulfonated monoalkylated benzene, wherein the alkyl group contained around fourteen carbon atoms, was substituted for the sodium sulfonate of tetradecyl phenol set forth in that example. This aqueous solution was circulated through the cooling system in the manner indicated in Example 1. Substantially the same results were secured.

This application is a continuation-in-part of my copending application, Serial No. 78,542, for "Cleaning composition and method for its use," filed May 8, 1936.

The invention is susceptible of modification within the scope of the appended claims.

I claim:

1. An acidic cleaning composition that is stable in solid form, and adapted in aqueous solution to remove scale, oxide impurities, grease and oil from ferrous and non-ferrous metal surfaces, while inhibiting acid attack upon surfaces of aluminum, brass, copper, tin and lead, which composition comprises a solid alkali metal salt of an inorganic acid adapted in aqueous solution to hydrolyze and yield a free acid; a solid water-soluble salt of a compound selected from the group consisting of the sulfonation products of alkylated phenols and cresols having between nine and sixteen carbon atoms in the alkyl group, the sulfonation products of alkylated benzene having between nine and sixteen carbon atoms in the alkyl group, and the sulfonation and sulfation products of monohydric aliphatic alcohols having between eight and seventeen carbon atoms in the molecule; and a small amount of a solid water-soluble phosphate corrosion inhibitor.

2. A cleaning composition that is stable in solid form and is acidic in aqueous solution, said composition being adapted in aqueous solution to remove scale, oxide impurities, grease and oil from ferrous and non-ferrous metal surfaces, while inhibiting acid attack upon surfaces of aluminum, brass, copper, tin and lead by said solution, which composition comprises a mixture in finely-divided solid form of a major portion of an alkali metal salt of an inorganic acid adapted in aqueous solution to yield a free acid; a water-soluble salt of a sulfonated derivative of a compound selected from the group consisting of the alkylated phenols and alkylated cresols wherein the alkyl group contains between nine and sixteen carbon atoms, the alkylated benzenes wherein the alkyl group contains between nine and sixteen carbon atoms, and the aliphatic monohydric alcohols having between eight and seventeen carbon atoms; and a small amount of a water-soluble phosphate effectively inhibiting the corrosion of non-ferrous metals by an aqueous solution of said composition.

3. A cleaning composition that is stable in solid form, and adapted in aqueous solution to remove scale, oxide impurities, grease and oil from ferrous and non-ferrous metal surfaces, while inhibiting acid attack upon surfaces of aluminum, brass, copper, tin and lead, which composition comprises a finely-divided solid mixture of a major portion of an alkali metal inorganic salt adapted in aqueous solution to hydrolyze and yield a free acid; a water-soluble salt of a sulfonated derivative of an alkylated phenol having between nine and sixteen carbon atoms in the alkyl group; and a small amount of a water-soluble phosphate effectively inhibiting the corrosion of non-ferrous metals by said com-

position in aqueous solution; said composition being substantially acidic in aqueous solution.

4. A cleaning composition that is stable in solid form, and adapted in aqueous solution to remove scale, oxide impurities, grease and oil from ferrous and non-ferrous metal surfaces, while inhibiting acid attack upon surfaces of aluminum, brass, copper, tin and lead, which composition comprises a mixture in finely-divided solid form of a major portion of an alkali metal salt of an inorganic acid adapted in aqueous solution to yield a free acid; a water-soluble salt of a sulfonated derivative of an alkylated benzene having between nine and sixteen carbon atoms in the alkyl group; and a small amount of a water-soluble phosphate effectively inhibiting the corrosion of non-ferrous metals by an aqueous solution of said composition; said composition being substantially acidic in aqueous solution.

5. A cleaning composition in solid form, adapted in aqueous solution to remove scale, oxide impurities, grease and oil from ferrous and non-ferrous metal surfaces while inhibiting acid attack upon surfaces of aluminum, brass, copper, tin and lead by said solution, which composition comprises a major portion of a water-soluble alkali metal bisulfate adapted in aqueous solution to release a free acid; a water-soluble salt of a sulfonated derivative of a compound selected from the group consisting of the aliphatic monohydric alcohols having between eight and seventeen carbon atoms, the alkylated phenols and alkylated cresols wherein the alkyl group contains between nine and sixteen carbon atoms, and the alkylated benzenes wherein the alkyl group contains between nine and sixteen carbon atoms; and a small amount of a solid water-soluble phosphate effectively inhibiting the corrosion of aluminum and other non-ferrous metals by an aqueous solution of the composition, said composition being acidic in aqueous solution.

6. A cleaning composition that is stable in solid form and is acidic in aqueous solution, and adapted in solution in water to remove scale, oxide impurities, grease and oil from ferrous and non-ferrous metal surfaces, while inhibiting acid attack upon surfaces of aluminum, brass, copper, tin and lead, which composition comprises a mixture of solid components comprising, by weight, about 85% of a water-soluble bisulfate adapted in aqueous solution to yield a free acid, about 6% of a water-soluble salt of a sulfonated derivative of a compound selected from the group consisting of the alkylated phenols and alkylated cresols wherein the alkyl group contains between nine and sixteen carbon atoms, the alkylated benzenes wherein the alkyl group contains between nine and sixteen carbon atoms, and the aliphatic monohydric alcohols having between eight and seventeen carbon atoms; and about 4% of a water-soluble phosphate effectively inhibiting the corrosion of non-ferrous metals by an aqueous solution of said composition, the balance being a water-soluble sulfate.

7. A cleaning composition that is stable in solid form and is acidic in aqueous solution, and adapted in aqueous solution to remove scale, oxide impurities, grease and oil from ferrous and non-ferrous metal surfaces while inhibiting acid attack upon surfaces of aluminum, brass, copper, tin and lead, which composition comprises a mixture of solid components comprising by weight about 85% of a water-soluble bisulfate adapted in aqueous solution to yield a free acid, about 6% of a water-soluble salt of a sulfonated derivative

of an alkylated phenol having between nine and sixteen carbon atoms in the alkyl group, and about 4% of dibasic ammonium phosphate, the balance being a water-soluble sulfate.

8. A cleaning composition that is stable in solid form and is acidic in aqueous solution, and adapted in aqueous solution to remove scale, oxide impurities, grease and oil from ferrous and non-ferrous metal surfaces, while inhibiting acid attack upon surfaces of aluminum, brass, copper, tin and lead, which composition comprises a mixture of solid components comprising, by weight, about 85% of a water-soluble bisulfate adapted in aqueous solution to yield a free acid, about 6% of a water-soluble salt of a sulfonated derivative of an alkylated benzene having between nine and sixteen carbon atoms in the alkyl group, and about 4% of dibasic ammonium phosphate, the balance being a water-soluble sulfate.

9. An acidic cleaning composition adapted to remove scale, oxide impurities, grease and oil from ferrous and non-ferrous metal surfaces, while inhibiting acid attack upon surfaces of aluminum, brass, copper, tin and lead, which composition comprises an aqueous solution containing approximately from 0.1% to 10% of a free inorganic acid; from 0.01% to 1% of a water-soluble salt of a sulfonated derivative of a compound selected from the group consisting of the aliphatic monohydric alcohols having between eight and seventeen carbon atoms, the alkylated phenols and alkylated cresols wherein the alkyl group contains between nine and sixteen carbon atoms, and the alkylated benzenes wherein the alkyl group contains between nine and sixteen

5 carbon atoms; and a water-soluble phosphate in amount sufficient to provide in said solution a phosphate ion concentration of between 0.05% and 0.5%; and water.

10 10. The method of cleaning metal surfaces, portions of which are formed of non-ferrous metals such as aluminum, brass, copper, tin and lead, while inhibiting the corrosion of said metals, which comprises applying to said metal surfaces, while heating the same, an acidic aqueous solution formed by mixing with water an alkali metal bisulfate, a water-soluble organic sulfonation product, and secondary ammonium phosphate; said water-soluble sulfonation product essentially comprising a solid water-soluble salt of a compound selected from the group consisting of the sulfonation products of alkylated phenols and cresols having between nine and sixteen carbon atoms in the alkyl group, the sulfonation products of alkylated benzene having between nine and sixteen carbon atoms in the alkyl group, and the sulfonation and sulfation products of monohydric aliphatic alcohols having between eight and seventeen carbon atoms in the molecule; the said solution having an effective free acid concentration of between 0.1% and 10%, from 0.01% to 1% of said water-soluble sulfonation product, and a phosphate group concentration of between 0.05% and 0.5%; thereafter withdrawing said solution from contact with the cleaned surfaces, and neutralizing at least the major part of any residual solution in contact with said surfaces.

TIMOTHY J. COLEMAN.